# EUROPEAN PATENT SPECIFICATION

(11) **EP 1 078 774 B1**
(45) Date of publication and mention of the grant of the patent: **03.11.2004**
(21) Application number: 00306610.7
(22) Date of filing: 03.08.2000
(51) Int. Cl.: B41M 5/00

(54) **Technique for modifying the coefficient of friction of inkjet media**
Verfahren um den Reibungsbeiwert von Tintenstrahl-Empfangsmaterialien zu modifizieren
Technique pour modifier le coefficient de friction de récepteurs pour l'impression au jet d'encre

(30) Priority: 26.08.1999 US 383884
(43) Date of publication of application: 28.02.2001
(73) Proprietor: Hewlett-Packard Company, A Delaware Corporation, Palo Alto, CA 94304 (US)
(72) Inventor: Sheng, Minghui, Cupertino, CA 95014 (US); Burch, Eric, San Diego, CA 92127 (US); Macleod, Cheryl A., Ramona, CA 92065 (US)
(74) Representative: Carpmaels & Ransford

(56) References cited:
- EP-A- 0 742 107
- EP-A- 0 819 990
- US-A- 4 713 280
- US-A- 5 700 582

## Description

### BACKGROUND OF THE INVENTION

The present invention relates generally to ink jet media and, more particularly, to techniques for modifying the coefficient of friction of such media.

The need for coated paper is well established. Paper may be coated with polymeric or wax coatings for various reasons such as for imparting water resistance, increasing strength of paper stock, enhancing gloss and improving barrier qualities.

The selection of coatings for the paper media utilized in modern image transfer devices, including ink jet printers, presents several problems. For example, because of the necessity that such coatings be capable of absorbing water based inks, the coatings tend to be softened by water or humidity. As a result, when two of these coatings are in contact, interaction between soft polymer coatings tends to be high and some sticking results. This factor can present significant problems feeding a single sheet from a paper stack to a printer is desired. In addition, humidity in some cases can contribute to a tacky feeling which is not aesthetically pleasing to the user and which can make the paper relatively difficult to handle.

Many of the pigments utilized in conventional ink jet coatings are characterized by high coefficients of friction. In fact, the silica and alumina pigments frequently utilized are referred to as "frictionizers". Further, since it is often desirable that the media have a smooth texture and glossy consistency, the techniques utilized to achieve these characteristics often produce media having high coefficients of friction.

As mentioned, media having a high coefficient of friction can be troublesome in sheet feeding printer operations because of the tendency of one sheet to stick to another. The coefficient of friction problem becomes particularly troublesome when a glossy ink jet coating is desired on both sides of the media, in order to support two sided printing.

Some prior art solutions to the above described problems have been attempted. In US patent no. 5,700,582, for example, backing materials are placed on a media substrate to reduce electrostatic charge and to reduce sheet to sheet friction and sticking. While this approach may have value in some cases, it is not suitable for media intended for two sided printing.

US patent no. 5,474,843 discloses the use of polymeric beads sticking through the surface of the media coating to improve sheet feeding properties. This solution is not compatible with some modern paper production processes. For example, it is not acceptable in a coating doctoring process to have particulates catch on the doctoring apparatus with scratches thereby produced in the coating. Calendaring or other smoothing processes will also diminish the utility of this technique, as the polymeric beads tend to be pushed into the coating.

From the foregoing it is apparent that there is a need for glossy ink jet media coatings that are compatible with modern inks and that have a low coefficient of friction to enable efficient sheet feeding functions.

Desirably, as an additional benefit, such media coatings would have a non-tacky consistency for good handleability.

EP-A-0,742,107 describes an ink jet recording medium comprising a plain paper base having, on one side, a porous ink-receiving layer that is smoother than that of the base and, on the other side, a coating layer comprising an aqueous binder containing 10 to 40% by weight of a higher fatty acid salt. The ink-receiving layer may comprise pigments, such as amorphous silica, water-soluble resin binders having satisfactory film-forming properties, such as PVA and polymer latices, and additives, such as cationic resins for improvement of water resistance, photo stabilizers for improvement of light resistance, and fluorescent brightening agents for improvement of whiteness. The aqueous binders used in the coating layer may include starch derivatives, such as oxidized starch and esterified starch, cellulose derivatives, such as carboxymethyl cellulose and hydroxyethyl cellulose, PVA and its derivatives, polyvinylpyrrolidone, casein, gelatin, styrene-butadiene latices, acrylate emulsions, styrene-acrylate emulsions, and vinyl acetate emulsions.

To prevent the feed roll from slipping, the coefficient of dynamic friction between two ink-receiving layers must be at least 0.65. To prevent discharge roll slippage, the coefficient of dynamic friction between two coating layers must be at least 0. 15. To ensure that the coefficient of static friction between the ink-receiving layer and the coating layer is less than 0.65, which is necessary to prevent double-feeds, the coefficient of dynamic friction between two ink-receiving surfaces must not exceed 0.75 and the coefficient of dynamic friction between two coating layers must not exceed 0.25. The ink-receiving layers and the coating layers are different in composition.

EP-A-0,819,990 describes a reclaimable transparency comprising a transparent base sheet coated on at least one side with a transparent, toner-receptive coating. The coating comprises from 60% to 85% of a polymeric antistatic binder composition, from 5% to 20% of a glycidoxy silane; from 3% to 12% of a wax; and from 3% to 15% of a particulate material having a mean particle size of from 4 µm to 15 µm.

### SUMMARY OF THE INVENTION

According to the present invention, there is provided ink jet media, comprising an opaque substrate having two sides and a glossy, water-based coating on both sides of said substrate for enabling water-based ink absorption and including a binder comprising between 5% and 30%, by weight, of said coating, a pigment selected from the group consisting of alumina and silica and a low friction substance in an emulsified form, mixed with said binder and selected from the group consisting of waxes, non-ionic polyethylene, silicone polymers and fluoro-polymers.

A method of preparing ink jet media from an opaque substrate having two sides of the present invention comprises mixing together a binder, a pigment selected from the group consisting of alumina and silica, and an emulsified form of a low friction substance selected from the group consisting of waxes, non-ionic polyethylene, silicone polymers and fluoro-polymers and applying the mixture to both sides of an opaque substrate to form a glossy, water-based coating for enabling water-based ink absorption in which the binder comprises between 5% and 30%, by weight, of said coating. The present invention affords several advantages over conventional media coating techniques. For example, it utilizes low friction materials in an emulsified form to decrease the coefficient of friction of a two-sided ink jet coating. In general, low friction materials may be described as waxes, simple organic polymers, silicone polymers or fluorinated polymers. The use of these materials in an emulsified form allows easy incorporation into a water-based coating. This technique is novel and original since it is generally believed that these materials do not function at high concentrations in an ink jet coating because of their hydrophobic nature, which suggests poor wetting and adsorptivity of water based inks. In this regard, it has been discovered that the use of low-friction materials allows a decrease of sheet coefficient of friction without degrading image quality.

In addition, the examples set forth herein support the hypothesis that the preparation of the coating materials in emulsion form imparts desirable properties to the media when contacted with ink jet ink.

Other aspects and advantages of the present invention will become apparent from the following detailed description, illustrating by way of example the principles of the invention.

### BEST MODE FOR CARRYING OUT THE INVENTION

The present invention may be embodied in other specific forms without departing from its essential characteristics. The described embodiments are to be considered in all respects only as illustrative and not restrictive. The scope of the invention is, therefore, indicated by the appended claims rather than by the foregoing description.

A preferred embodiment of the present invention provides glossy ink jet media coatings that are compatible with modern inks and have a low coefficient of friction, to enable efficient sheet feeding functions. The inventive technique enables effective and efficient two-sided copying wherein both paper sides utilize glossy coatings having a low coefficient of friction. In this manner, improved ink retention is achieved while sheet-feeding problems are substantially reduced.

In a preferred embodiment, an ink jet media coating comprises a substrate including a binder and a low friction, in an emulsified form, selected from the group consisting of waxes, simple organic polymers, silicone polymers and fluoropolymers. Preferably, polyterfluoroethylene latex is utilized as a slip aid. The binder is selected from the group consisting of polyvinylversatate, polyethelene, polyvinyl alcohol, polyvinylpyrrolidone and polyvinylacetate and it comprises between about 5% and about 30%, by weight, of the coating.

A method of preparing ink jet media of the present invention includes the steps of providing a substrate and a binder as described above. The binder is mixed with a low friction substance, in an emulsified form, selected from the group consisting of waxes, simple organic polymers, silicone polymers and fluoropolymers. The mixture is applied to the substrate and the substrate is dried.

In the presently preferred embodiment, the slip aid is a dispersion in water and preferably, is polymeric. The particle size of the dispersion is less than 5 µm, or preferably, less than 1 µm. While a variety of functional groups are feasible, the preferred slip aid mainly includes the elements carbon, hydrogen, fluorine, silicon or the "oxo" form of oxygen for maintaining desired friction properties. These elements are found in waxes, simple organic polymers, silicone polymers and fluoridated polymers. In general, a number of latex dispersions may be classified as slip aids. Polyterfluoroethylene latex, available from E.I. duPont de Nemours and Co. under the trademark Zonyl® TE-3667N, and a high molecular weight polyethylene wax, available from Shamrock Technologies, Inc., Newark, NJ under the designation Hydrocer-355, have proven effective. Other suitable slip aids are a nonionic polyethylene emulsion sold by Air Products and Chemicals, Inc., Allentown, PA, as Vancryl® Wax 35 and a carnauba wax produced by Michelman, Inc., Cincinnati, Ohio, under the trademark MICHEM® LUBE 160.

According to the present invention, an ink jet coating is applied to a substrate by conventional methods. Typically, the coating includes pigment, binder and performance additives. A preferred pigment is psuedo-boehmite alumina, manufactured by Condea-Vista as Dispal 11 N7-80. Its particle size in water is about 0.25µm while dried particle size is about 50µm.

In a preferred embodiment, the binders are polyvinylversatate polyethylene, present as a non-water soluble emulsion polymer, polyvinylalcohol and polyvinylpyrrolidone polyvinylacetate copolymer. The latter two are water soluble. These binders are present in dry solid weight percents of 2%, 0.6% and 11%, respectively. The polyvinylversatate polyethylene copolymer is manufactured by Mapei, Inc. of Canada, as Vinavil® 3525. The polyvinylalcohol is manufactured by Air Products and Chemicals, Inc., as Airvol® 165 and polyvinylpyrrolidone polyvinylacetate copolymer is available from Badische Anilin & Soda-Fabrik Aktiengesellschaft, Germany, under the trademark Luviskol®.

Performance additives are utilized for several reasons. For example, to control bleed and uniformity, diamine ethylene/propylene oxide surfactant, manufactured by BASF Corp. as Tetronic™ 701 and glycol, manufactured by Aldrich Chemical, are utilized. An organic acid, such as lactic acid manufactured by Aldrich, functions as a performance additive to control viscosity and bleeding. A silicon ether surfactant, manufactured by Air Products as Surfonyl™ D-58 serves as a performance additive to reduce foam. Finally, the performance additive polyterfluoroethylene latex, manufactured by E. I. DuPont de Nemours and Co. as Zonyl® TE-3667N, functions as a slip aid.

TABLE I sets forth the composition of a low cost, glossy ink jet coating, prepared according to the present invention and having a relatively low coefficient of friction.

**TABLE I**

| Chemical | General Class | Parts | Percent |
|---|---|---|---|
| Boehmite alumina | Pigment | 100 | 78.40063 |
| Polyvinylversatate Polyethylene copolymer | Binder | 14.4 | 11.28969 |
| Polyvinylalcohol | Binder | 0.8 | 0.627205 |
| Polyvinylpyrrolidone polyvinylacetate copolymer | Binder | 2.9 | 2.273618 |
| Diamine ethylene/propylene oxide surfactant | Performance additive | 1.1 | 0.862407 |
| Glycol | Performance additive | 1.3 | 1.019208 |
| Lactic acid | Performance additive | 1 | 0.784006 |
| Silicon ether surfactant | Performance Additive | 0.05 | 0.0392 |
| Polyterfluoroethylene latex | Slip aid | 6 | 4.7040938 |

In order to demonstrate the utility of the present invention, ink jet coatings formulated according to the present invention were tested. The examples that follow illustrate certain specific embodiments of the invention and describe comparative tests with commercially available ink jet media coatings.

### EXAMPLE 1

A coating was prepared that contained the substances set forth in TABLE I. The materials were mixed together and then coated on a clay-coated base sheet using a mayer rod. The sheet was dried for 5 minutes at 100° C and then calendared until glossy. The constituents of the coating of Example I are set forth in TABLE II.

**TABLE II**

| Chemical | Manufacturer | Grade | Parts (Dry wgt.) |
|---|---|---|---|
| Pigment | Condea Vista | Dispal 11N7-80 | 100 |
| Polymer | ISP | PVPVA-7/30 | 3 |
| Polymer | Air Products and Chemicals, Inc. | Airvol® 165 | 1 |
| Polymer | Vinavil | 3525 | 15 |
| Plastisizer | Aldrich Chemical | Glycerol Reagent | 2 |
| Surfactant | BASF Corp. | Tetronic™ 701 | 1 |
| Surfactant | Air Products | Surfonyl DF-58 | 0.05 |
| Acid | Aldrich Chemical | Lactic Acid Reagent | 1 |
| Slip-aid | E.I DuPont de Nemours & Co. | Polyterfluoro ethylene latex | 6 |

### EXAMPLE 2

A second coating was prepared and a glossy sheet was produced by the method set forth in Example 1. The second coating was identical to the Example 1 coating except that 6 parts of Shamrock Hydrocer-355 (waxy polymer) were utilized as a slip aid instead of polyterfluoroethylene latex (Zonyl® TE-3667).

### EXAMPLE 3

A third coating was prepared and a glossy sheet was produced by the method set forth in Example 1. The coating utilized in this example is conventional. It is similar to the coatings of Examples 1 and 2 but differed therefrom by having neither the polyterfluoroethylene latex (Zonyl® TE-3667) of Example 1 nor the Shamrock Hydrocer-355 polyfluoroethylene polymer of Example 2.

Comparative tests were conducted on the coatings produced in the examples. The results are set forth in TABLE III.

**TABLE III**

| Results | Example 1 | Example 2 | Example 3 |
|---|---|---|---|
| 60 degree gloss | <40% | <40% | <40% |
| IQ (HP 890C) | high | high | high |
| Static CoF | 0.50 | 0.48 | 0.75 |
| Kinetic CoF | 0.35 | 0.35 | 0.77 |
| Printed Static CoF | 0.67 | 0.56 | 0.76 |
| Printed Kinetic CoF | 0.42 | 0.37 | 0.77 |

As can be seen from the results set forth in TABLE III, the use of the slip aid in Examples 1 and 2 enables the production of a glossy sheet having excellent print quality. In addition, the coefficient of friction is substantially reduced in the coatings of Examples 1 and 2, in comparison to the conventional coating of Example 3. As a result, ink jet media having reliable sheet feeding properties are produced. In addition, the media do not feel tacky when handled.

## Claims

1. Ink jet media, comprising:
an opaque substrate having two sides; and
a glossy, water-based coating on both sides of said substrate for enabling water-based ink absorption and including:
a binder comprising between 5% and 30%, by weight, of said coating;
a pigment selected from the group consisting of alumina and silica; and
a low friction substance in an emulsified form, mixed with said binder and selected from the group consisting of waxes, non-ionic polyethylene, silicone polymers and fluoropolymers.

2. The ink jet media according to claim 1, wherein said binder is selected from the group consisting of polyvinylversatate, polyethylene, polyvinyl alcohol, polyvinylpyrrolidone and polyvinylacetate.

3. The ink jet media according to claim 1 or claim 2, wherein said low friction substance is selected from the group consisting of polyterfluoroethylene latex, high molecular weight polyethylene wax, non-ionic polyethylene emulsions and carnuba wax.

4. A method of preparing ink jet media from an opaque substrate having two sides, comprising:
mixing together a binder, a pigment selected from the group consisting of alumina and silica, and an emulsified form of a low friction substance selected from the group consisting of waxes, non-ionic polyethylene, silicone polymers and fluoro-polymers; and
applying the mixture to both sides of an opaque substrate to form a glossy, water-based coating for enabling water-based ink absorption in which the binder comprises between 5% and 30%, by weight, of said coating.

5. The method according to claim 4, wherein the binder is selected from the group consisting of polyvinylversatate, polyethylene, polyvinyl alcohol, polyvinylpyrrolidone and polyvinylacetate.

## Patentansprüche

1. Tintenstrahlmedium, das folgende Merkmale aufweist:
ein undurchsichtiges Substrat, das zwei Seiten aufweist; und
eine auf Wasser basierende Glanzbeschichtung auf beiden Seiten des Substrats, um eine Absorption von auf Wasser basierender Tinte zu ermöglichen, wobei die Beschichtung folgende Merkmale umfasst:
ein Bindemittel, das zwischen 5 und 30 Gewichtsprozent der Beschichtung ausmacht;
ein Pigment, das aus der Gruppe ausgewählt ist, die aus Aluminiumoxid und Silika besteht; und
eine reibungsarme Substanz in emulgierter Form, die mit dem Bindemittel gemischt ist und aus der Gruppe ausgewählt ist, die aus Wachsen, nicht-ionischem Polyethylen, Silikonpolymeren und Fluorpolymeren besteht.

2. Das Tintenstrahlmedium gemäß Anspruch 1, bei dem das Bindemittel aus der Gruppe ausgewählt ist, die aus Polyvinylversatat, Polyethylen, Polyvinylalkohol, Polyvinylpyrrolidon und Polyvinylacetat besteht.

3. Das Tintenstrahlmedium gemäß Anspruch 1 oder 2, bei dem die reibungsarme Substanz aus der Gruppe ausgewählt ist, die aus Polyterfluorethylenlatex, Polyethylenwachs mit hoher relativer Molekülmasse, nichtionischen Polyethylenemulsionen und Karnaubawachs besteht.

4. Ein Verfahren zum Herstellen eines Tintenstrahlmediums aus einem undurchsichtigen Substrat, das zwei Seiten aufweist, wobei das Verfahren folgende Schritte umfasst:
Miteinandervermischen eines Bindemittels, eines Pigments, das aus der aus Aluminiumoxid und Silika bestehenden Gruppe ausgewählt ist, und einer emulgierten Form einer reibungsarmen Substanz, die aus der Gruppe ausgewählt ist, die aus Wachsen, nicht-ionischem Polyethylen, Silikonpolymeren und Fluorpolymeren besteht; und
Aufbringen des Gemischs auf beide Seiten eines undurchsichtigen Substrats, um eine auf Wasser basierende Glanzbeschichtung zu bilden, um eine Absorption von auf Wasser basierender Tinte zu ermöglichen, wobei das Bindemittel zwischen 5 und 30 Gewichtsprozent der Beschichtung ausmacht.

5. Das Verfahren gemäß Anspruch 4, bei dem das Bindemittel aus der Gruppe ausgewählt ist, die aus Polyvinylversatat, Polyethylen, Polyvinylalkohol, Polyvinylpyrrolidon und Polyvinylacetat besteht.

## Revendications

1. Support à jet d'encre comprenant :
un substrat opaque présentant deux faces ; et
un revêtement brillant à base d'eau sur les deux faces dudit substrat permettant l'absorption d'encre à base d'eau et comprenant :
un liant comprenant entre 5 % et 30 % en poids dudit revêtement ;
un pigment sélectionné dans le groupe constitué de l'alumine et de la silice ; et
une substance à coefficient de frottement réduit sous une forme émulsifiée, mélangée avec ledit liant et sélectionnée dans le groupe constitué des cires, du polyéthylène non ionique, des polymères de silicone et des fluoropolymères.

2. Support à jet d'encre selon la revendication 1, dans lequel ledit liant est sélectionné dans le groupe constitué du polyvinylversatate, du polyéthylène, de l'alcool de polyvinyle, de la polyvinylpyrrolidone et du polyvinylacétate.

3. Support à jet d'encre selon la revendication 1 ou la revendication 2, dans lequel ladite substance à coefficient de frottement réduit est sélectionnée dans le groupe constitué du latex de polyterfluoroéthylène, de la cire de polyéthylène à poids moléculaire élevé, des émulsions de polyéthylène non ionique et de la cire de carnuba.

4. Méthode de préparation d'un support à jet d'encre à partir d'un substrat opaque présentant deux faces, comprenant :
le mélange d'un liant, d'un pigment sélectionné parmi le groupe constitué de l'alumine et de la silice, et d'une forme émulsifiée d'une substance à coefficient de frottement réduit sélectionnée parmi le groupe constitué des cires, du polyéthylène non ionique, des polymères de silicone et des fluoropolymères ; et
l'application du mélange sur les deux faces d'un substrat opaque afin de former un revêtement brillant à base d'eau permettant l'absorption d'encre à base d'eau dans lequel le liant comprend entre 5 % et 30 %, en poids, dudit revêtement.

5. Méthode selon la revendication 4, dans laquelle le liant est sélectionné dans le groupe constitué du polyvinylversatate, du polyéthylène, de l'alcool de polyvinyle, de la polyvinylpyrrolidone et du polyvinylacétate.
